

# UNITED STATES PATENT OFFICE.

FREDERICK M. BECKET, OF NIAGARA FALLS, NEW YORK, ASSIGNOR TO ELECTRO METALLURGICAL COMPANY, OF NIAGARA FALLS, NEW YORK, A CORPORATION OF WEST VIRGINIA.

## ALLOY.

1,322,158.

Specification of Letters Patent. Patented Nov. 18, 1919.

No Drawing.

Application filed June 7, 1918. Serial No. 238,726.

To all whom it may concern:

Be it known that I, FREDERICK M. BECKET, a subject of the King of Great Britain, residing at Niagara Falls, in the county of 5 Niagara and State of New York, have invented certain new and useful Improvements in Alloys, of which the following is a specification.

This invention comprises a novel alloy, 10 useful for various purposes, but more particularly in connection with the deoxidation and purification of steel or iron, and the production of alloy-steels. The alloy contains as its essential components magnesium and silicon, and preferably manganese. Other metals, including iron, may also be present. In the preferred composition of 15 the alloy the magnesium is present in excess of the molecular proportion to the silicon. The invention comprises also the process involved in the treatment of molten iron and steel with such alloys.

It is well known that magnesium is a most efficient deoxidizing agent for steel, 20 but its reactivity is such as to render its introduction in the pure or un-alloyed state into molten steel a matter of extreme difficulty. Moreover the melting point of the resulting slag is so high as to render its 25 elimination difficult. Silicon in material proportions not only moderates the violence of the magnesium-oxidation reaction, but when the silicon is properly proportioned to the magnesium its oxidation product unites with that of magnesium to yield a 30 relatively fusible and hence much more easily eliminated slag. It is believed that silicon, used in conjunction with sufficient proportions of magnesium, tends also to a better 35 elimination of the sulfur, due to the fact that the oxidation of magnesium raises the temperature of the melt to a point at which the known desulfurizing action of silicon becomes efficient.

40 Alloys containing 50-90 per cent. of magnesium; 10-40 per cent. of silicon; and up to 10 per cent. of iron, are eminently adapted for the treatment of steel. In such alloys the proportion of magnesium, rela-

tive to the silicon, is higher than corresponds to the so-called silicid of magnesium,  $MgSi$ ; that is to say, the magnesium is in excess of the equimolecular proportion of the silicon. This is true irrespective of whether other metals, including iron and manganese, enter into the constitution of the alloys.

I have found that such alloys, in contradistinction to the calcium-silicon compounds containing more calcium than corresponds to the equimolecular proportion indicated by the formula  $CaSi$ , are sufficiently stable for the purpose in view.

I prefer to introduce into the alloy a sufficient proportion of manganese to further reduce the melting point of the slag, which in this case is essentially a magnesium-manganese-silicate. The proportion of manganese in the alloy may be such as to introduce any desired quantity of this metal into 70 the alloy steel. A typical alloy of this type may comprise, together with other components if desired:

|           |           |    |
|-----------|-----------|----|
| Magnesium | 50-70%    | 75 |
| Silicon   | 10-20%    |    |
| Manganese | 10-20%    |    |
| Iron      | up to 10% |    |

The iron is not regarded as an essential component of either alloy, but its presence 80 is more or less incidental to the employment of a high grade ferrosilicon as a convenient means of introducing the required amount of silicon into the alloy. In like manner the manganese may be supplied as ferro- 85 manganese, with the resulting introduction of further quantities of iron into the alloy.

I claim:

1. An alloy containing as essential components magnesium, silicon and manganese, 90 the magnesium in excess of the equimolecular proportion to the silicon.

2. An alloy containing approximately magnesium 50-90 per cent.; silicon 10-20 per cent.; manganese 10-20 per cent. and 95 iron up to 10 per cent.

3. Process of treating molten steel or iron for the purification thereof or the produc-

tion of alloy steels, which consists in introducing thereinto an alloy containing magnesium and silicon, the magnesium in excess of the equimolecular proportion to the silicon.

4. Process of treating molten steel or iron for the purification thereof or the produc-

tion of alloy steels, which consists in introducing thereinto an alloy containing magnesium, silicon and manganese, the magnesium in excess of the equimolecular proportion to the silicon. 10

In testimony whereof I affix my signature.  
FREDERICK M. BECKET